

## UNITED STATES PATENT OFFICE.

CHARLES M. NOKES, OF SALT LAKE CITY, UTAH, ASSIGNOR TO EUREKA METALLURGICAL COMPANY, OF SALT LAKE CITY, UTAH.

## FLOTATION PROCESS AND COMPOSITION.

No Drawing.

Application filed March 4, 1922. Serial No. 541,207.

*To all whom it may concern:*

Be it known that I, CHARLES M. NOKES, a citizen of the United States, residing at Salt Lake City, in the county of Salt Lake 5 and State of Utah, have invented certain new and useful Improvements in Flotation Processes and Compositions, of which the following is a specification.

This invention relates to an improvement 10 in the flotation process of and composition for recovering values from ore, particularly non-sulfide ores, and among the objects of the invention are to make the desired particles of such ores subject or more amenable 15 to concentration by flotation.

More or less specifically stated, the invention consists in mixing certain addition agents intimately together before introducing them into the pulp, these addition 20 agents having the function of assisting in the subsequent flotation action, by acting upon oxidized or non-sulfide ores, or a mixture of sulfide and non-sulfide ores to make the non-sulfide portion float in the subsequent 25 flotation stage, making the lifting oils more effective, etc.

In a typical instance of the use of my process, I employ in the preparation stage, a solid hydrocarbon, such as paraffin, and 30 an alkaline sulfide, such as sodium-sulfide, the ore under treatment being a non-sulfide ore, or a mixture of sulfide and non-sulfide ores. The paraffin and the sodium-sulfide are fused or mixed together at a temperature 35 sufficiently high to permit of the liquefaction of the hydrocarbon. To effect this I may pulverize the sodium-sulfide to say 100 to 250 mesh. I next melt the paraffin, and then make a paste by mixing the paraffin 40 and the pulverized sodium-sulfide. This paste, as it cools, solidifies into an apparently homogeneous mass. If this be allowed to solidify without stirring, it becomes hard and flinty and must be pulverized 45 before addition to the tube mill. But stirring seems to give it a more or less granular condition, somewhat lumpy, and suitable when broken into fragments, for the tube mill. It is introduced into the tube mill along with the ore, to be ground into pulp, or it may be introduced into the pulp 50

after the ore has been ground and passed to emulsifiers.

It should be understood that this mixture is not a froth or scum maker, or "lifter", 55 and therefore other oils are added, such as pine oils, to expedite the formation of a certain amount of froth or scum wherein the particles of the mixture collect and with which they may be removed from the 60 flotation cell. The function of the paraffin-sodium-sulfide mixture is one of preparation, and not one of flotation or frothing. It acts upon non-sulfide or oxidized 65 ores so that in the flotation stage they float, while the gangue remains submerged. Certain lifting oils, like Yaryan pine, which will not lift oxidized ores direct, will do so after the addition of the paraffin mixture. 70 If the lifting oils were omitted, the paraffin-sodium-sulfide mixture alone would give flotation in the flotation stage, but the scum would be too sparse to remove with sufficient rapidity; it would be very sparse and very rich, made up of a vast number of 75 particles of paraffin of minutest size, each one solid and with the mineral particles or values clinging to it.

The amounts of the mixture employed, and the ratios between paraffin and sodium-sulfide vary. On oxidized copper ores I have used six to ten pounds, per ton of ore, of sodium sulfide, and the same amount of paraffin. On other ore I have used ten pounds of the sodium sulfide and seven and one-half pounds of paraffin. In this case I used thirteen pounds per ton of ore of the lifting oils, etc.

Experiment showed that when the two components of this mixture, that is to say sodium-sulfide and paraffin, were added to the pulp simultaneously or successively but separately, not as good results were obtained as when added in the way I have indicated. Maximum effectiveness seems to be due to 90 the intimate association of the two components before they are added to the pulp. I have stated that the mixture may be best accomplished by pulverizing the sodium-sulfide very finely and mixing it with melted 95 paraffin, and at a temperature such that the sodium-sulfide is not fused. If the sodium 100

sulfide is fused it has a tendency to liqueate away from the paraffin. Other methods of procedure may be, simply grinding the two ingredients together, heating them very 5 highly and spraying them into the pulp, etc.

The process is economical in so far as materials are concerned, because the paraffin and oils may be subsequently recovered by 10 heating with water. I also find that with the use of this mixture demineralization of the pulp is much more rapid. It will be understood that though I have referred specifically to sodium-sulfide and paraffin, I 15 do not intend any limitation to the use of these particular materials. I do believe that a solid hydrocarbon is essential, that is, a hydrocarbon which is in the solid state, or in a state approaching solidity, under the 20 normal temperatures of pulp preparation and flotation. Paraffin and slack wax are examples of such hydrocarbons, but when I mention solid hydrocarbons I mean hydrocarbons having the same or equivalent characteristics 25 for the purposes of my process. And, of course, I might use some other reagent than sodium sulfide, provided that it could be employed with a solid hydrocarbon in preparing non-sulfide ore for effective flotation.

The following are examples of the practical application of my invention:

*Example No. 1.*

35 500 grams of a silver ore containing manganese was mixed with 500 c. c. of water and a mixture consisting of 2.5 grams of sodium sulfide and 1.75 grams of paraffin, and  $\frac{1}{8}$  gram of reconstructed Yaryan pine 40 oil, ground in a ball mill until 80% of the ore passed an 80-mesh screen.

The pulp was removed from the tube mill and allowed to settle. The excess water was decanted and the remaining pulp was poured 45 into a laboratory flotation machine and 1200 c. c. of fresh water added, and also 0.25 grams of reconstructed Yaryan pine oil, and 0.75 grams of a mixture of 50% benzol, 20% reconstructed Yaryan, and 30% P. and E. 50 oil (a petroleum oil). The dilute pulp was then agitated and the concentrates removed. The ore contained 0.24 ozs. gold, 33.36 ozs. silver, and 4.33% manganese. The concentrates assayed 3.50 ozs. gold, 374.0 ozs. silver, 55 and 4.50% manganese. The tailings assayed

0.04 ozs. gold, 4.96 ozs. silver, showing a recovery of 84.3% of the gold and 87% of the silver.

*Example No. 2.*

60

A thoroughly oxidized complex ore gave the following results:—

500 grms. of ore were mixed with 500 c. c. of water and a mixture of 2.5 grms. of sodium sulfide and 0.75 grms. of paraffin and  $\frac{1}{8}$  grm. of reconstructed Yaryan and 1.25 grms. of P. and E. oil. This mixture was ground in a tube mill for 20 minutes.

The pulp was allowed to settle and the excess water decanted. The remaining pulp was poured into a flotation machine and 1200 c. c. of water added, the pulp agitated and the concentrates removed. The tailings were then separated into sands and slimes, and each product agitated separately in the flotation machine and the concentrates removed.

The complete results are as follows:—

The ore assayed 0.04 ozs. gold, 30.94 ozs. silver, 6.65% lead and 1.63% copper.

80

The combined concentrates assayed 0.225 ozs. gold, 324.3 ozs. silver, 47.4% lead, and 5.0% copper. The combined final tailings assayed—trace gold, 1.76 ozs. silver, 0.50% lead and 0.31% copper, showing a recovery 85 of 90% gold; 95.0% silver; 93.5% lead and 86.5% copper.

I claim:

1. The process of preparing non-sulfide ore for concentration by flotation, which consists in first intimately mixing, in a finely divided state, sodium sulfide and a solid hydrocarbon, and thereafter adding the mixture to finely divided non-sulfide ore, and making a pulp including the ore and the mixture.

2. The process which consists in first intimately mixing sodium sulfide and a solid hydrocarbon, and thereafter including the mixture, in a finely divided and dispersed 100 state, within a pulp of non-sulfide ore.

3. A reagent for use in the flotation of non-sulfide ores, comprising homogenous mass of intimately mixed sodium sulfide and a solid hydrocarbon.

In testimony whereof I affix my signature in presence of two witnesses.

CHARLES M. NOKES.

105

Witnesses:

L. R. MARTINATE, Jr.,  
WARREN STRATTON.